

Patented Aug. 3, 1926.

1,595,052

# UNITED STATES PATENT OFFICE.

GEORGE W. ACHESON, OF CALDWELL, NEW JERSEY.

## PROCESS OF DEFLOCCULATING SOLIDS.

No Drawing.

Application filed March 8, 1926. Serial No. 93,328.

This invention relates to the art of deflocculating solid bodies, and comprises a process whereby the deflocculation can be accomplished more readily, more rapidly and with greater yields than heretofore. The term "deflocculation" is used herein in its commonly accepted sense, as indicating the subdivision of solid bodies, such for instance as graphite, carbon black, clay, pigments, insecticides such as lead arsenate, sulfur, etc., etc. into particles of colloidal dimensions, by a process of prolonged attrition in presence of moisture and of an organic "deflocculating agent", which agent has the general properties of tannin and tannin-like bodies. Among such deflocculating agents, as heretofore used in this art, I may mention tannin, cutch, and extracts from roasted cereals or starchy bodies, usually employed in conjunction with ammonia. While all of these substances possess in common the property of deflocculating such solids as are mentioned above, they differ considerably among themselves, particularly with respect to rapidity of action and the stability of the resulting colloid.

In the operation of deflocculating as ordinarily practiced, the deflocculating agent disappears, wholly or substantially, from the aqueous or ammoniacal solution, being absorbed by the particles of the solid. It is observed however that if an excess of deflocculating agent be used, or if the process of attrition be too prolonged, re-flocculation sets in, the previously deflocculated or colloidal particles re-uniting into aggregates which are no longer of colloidal dimensions and subside when suspended in water. Heretofore it has been universal practice to avoid carefully such conditions as lead to re-flocculation in the mill such re-flocculation involving a limitation upon or even a reduction of the obtainable yield of particles of colloid dimensions; the result being, in the case of graphite for example, that only a relatively small proportion of the total charge can be deflocculated in a single operation. In a typical case the proportion of graphite deflocculated or converted into the colloidal state in course of a single passage through the mill is of the order of six or eight percent. This percentage differs of course with different materials subjected to the operation, and also with the particular deflocculating agent used.

According to my improved process in its preferred embodiment, I first add to the solid to be deflocculated, for example graphite in the form of a heavy paste, a relatively small proportion, say six percent by weight, of one of the known deflocculating agents, for example tannin, preferably together with a small amount of aqueous ammonia; and I subject the paste to attrition under the usual conditions until the deflocculating agent has been substantially adsorbed. I then repeat this operation, adding new portions of the deflocculating agent, a number of times, depending on the results sought; but always ultimately introducing sufficient deflocculating agent so that a thorough mixing operation, following the final addition of agent, will bring about the re-flocculation of most or all of the initially deflocculated solid. In a typical instance, where the material to be deflocculated was electric furnace graphite, and the deflocculating agent used was tannin, the total amount of agent added amounted to about eighteen percent of the dry weight of the graphite.

At this stage a substantial proportion, in some cases upward of 80%, of the initial charge has passed through the deflocculated stage, but had undergone re-flocculation. This however does not mean that the original physical condition of the solid has been restored; for the re-flocculated aggregates, being assemblies of particles which have once passed through the colloidal state, are extremely fragile, although not capable of being resolved again into their colloidal components by simple stirring.

I have discovered however that these re-flocculated aggregates may be resolved again into their component particles of colloid dimensions by treating them with certain deflocculating or peptizing agents other than those used in the initial stage of the process. Among such agents, which I will term peptizing agents in order to distinguish them from the deflocculating agents used in the first stage, I prefer to use infusions of grasses (Gramineæ) such as hay, straw and the like; although I may use other vegetable infusions capable of the same peptizing effect; or inorganic peptizing agents such as sodium silicate may be used. This peptization may be carried out in the same or other mill, and under essentially the same conditions as the initial deflocculating treat-

ment. The result of this treatment, involving an initial deflocculation carried through to partial or complete re-flocculation, and followed by peptization of the re-flocculated aggregates, is greatly to increase the ultimate yield of colloid, as well as to increase the rate at which it is prepared from the initial raw material.

I claim:

- 10 1. Process of treating solid bodies to prepare particles of colloidal dimensions, comprising deflocculating and re-flocculating the said solid by attrition with an organic de-

15 flocculating agent; and thereafter peptizing the re-flocculated aggregates.

2. Process of treating solid bodies to prepare particles of colloidal dimensions, comprising deflocculating and re-flocculating the said solid by attrition with an organic de-  
20 flocculating agent; and thereafter peptizing the re-flocculated aggregates by means of an infusion of a grass.

In testimony whereof, I affix my signature.

GEORGE W. ACHESON.